# EUROPEAN PATENT SPECIFICATION

(11) **EP 2 045 396 B1**
(45) Date of publication and mention of the grant of the patent: **09.03.2016**
(21) Application number: 07425611.6
(22) Date of filing: 02.10.2007
(51) Int. Cl.: E01F 9/688, E04H 12/22

(54) **Process for producing a traffic- and parking-preventing element made of rubber**
Verfahren zur Herstellung eines Verkehrs- und Parkverhinderungselements aus Kautschuk
Procédé pour la fabrication d'un élément en caoutchouc pour empêcher la circulation et le stationnement

(43) Date of publication of application: 08.04.2009
(73) Proprietor: Casei Eco System S.R.L., 15057 Tortona (AL) (IT); Sada2 S.R.L., 15067 Novi Ligure (AL) (IT)
(72) Inventor: Ferrarini, Marco, 15057 Tortona (AL) (IT)
(74) Representative: Garavelli, Paolo

(56) References cited:
- EP-A- 1 277 883
- DE-A1- 19 652 696
- FR-A- 2 833 682
- KR-A- 20020 006 404
- US-A1- 2003 125 425
- ANONYMOUS: "PRODUCTION COMMERCIALISATION de Matériaux en Caoutchouc Recyclé" INTERNET ARTICLE, [Online] 1 July 2004 (2004-07-01), XP002465845 Retrieved from the Internet: URL:http://web.archive.org/web/20040701125 215/http://www.php03.com/> [retrieved on 2008-01-23]
- ANONYMOUS: "BORNE HEXDALLE YOSTRA" INTERNET ARTICLE, [Online] 11 April 2004 (2004-04-11), XP002465846 Retrieved from the Internet: URL:http://web.archive.org/web/20040411041 839/http://hexdalle.com/yostra.htm> [retrieved on 2008-01-23]

## Description

The present invention refers to a process for producing a traffic- and parking-preventing element made of rubber granules.

It is known in the art to use rubber, above all recycled rubber in the form of granules, for producing road kerbs, traffic- and parking-preventing elements and traffic deviating elements, slowing-down hump bridges and other permanent or temporary road devices for safety and/or for delimiting forbidden spaces for parking, for pedestrian, bicycle and vehicle traffic. The use of rubber, above all rubber deriving from run-down vehicle tires, in fact allows a more efficient production of the above devices, at the same time resulting in a valid support for recycling policies, that are more and more up-to-date in almost all Countries in the world. Moreover, such rubber devices have the advantages of not rusting, not discolouring, not chipping and not generating damages, at most very small damages, to vehicles in case of slight impacts. Rubber devices therefore are an efficient solution for parkings and all areas with intense vehicle traffic and where conventional devices get frequently damaged.

XP 002465845 discloses such a rubber device.

The inconvenience of such rubber manufactured products however is their lightness with respect to similar manufactured products made of concrete, reinforced concrete or metallic materials, making them easily displaceable or removable. As remedy for such problem, the art proposes a rubber traffic deviating device secured onto the road surface or underground that, if it receives an impact from a vehicle when manoeuvring, gets distorted, without being subjected to damages or without damaging the vehicles themselves.

KR-A-20020006404 instead discloses safety or traffic delimiting devices produced by moulding foamed polypropylene in granules and reinforced by a metallic or plastic structure or by en external layer made of rubber or polyethylene adapted to guarantee that the devices keep their initial shape.

Object of the present invention is solving the above prior art problems by providing a process for producing a traffic- and parking-preventing element made of rubber granules, in particular recycled rubber, whose weight is increased with an inert weight-increasing material, thereby not requiring the use of separate metallic or plastic structures, as instead provided by the known prior art.

Another object of the present invention is providing a process for producing a traffic- and parking-preventing element made of rubber granules that, being the weight-increasing material mixed in the rubber amalgam, can be produced in a single moulding operation without producing and afterwards integrating separate metallic or plastic structures.

Moreover, an object of the present invention is providing a process for producing a traffic- and parking-preventing element made of rubber granules in which the weight-increasing material is mixed in the amalgam.

The above and other objects and advantages of the invention, as will result from the following description, are obtained with a process for producing a traffic- and parking-preventing element made of rubber as described in claim 1.

Preferred embodiments and non-trivial variations of the present invention are the subject matter of the dependent claims.

It will be immediately obvious that numerous variations and modifications (for example related to shape, sizes and parts with equivalent functionality) could be made to what is described, without departing from the scope of the invention as appears from the enclosed claims.

The present invention will be better described by some preferred embodiments thereof, provided as a nonlimiting example, with reference to the single enclosed drawing, in which FIG. 1 shows a top perspective view of a preferred embodiment of the traffic- and parking-preventing element produced according to the process of the present invention.

With reference therefore to FIG. 1, the traffic- and parking-preventing element 1 is composed of a solid body equipped with at least one bearing base 2, such solid body being formed of at least one amalgam moulded in a solid shape composed of a mixture of rubber granules (the amounts of which will obviously depend on the sizes and/or the shape of the traffic- and parking-preventing element 1 that has to be obtained), of at least one polyurethane resin and of at least one weight-increasing inert material.

In addition, in case a coloured traffic- and parking-preventing element 1 has to be obtained, the above amalgam could also contain at least one colouring paste in the most suitable amounts.

Alternatively, in order to obtain a coloured traffic- and parking-preventing element 1, it is obviously possible to provide for colouring only its external surface with any type of paint.

In order to more strongly link the various components of the traffic- and parking-preventing element 1 one with the other, this element 1 further comprises at least one internal reinforcing structure, preferably of the cage or trellis type (not shown), still more preferably made of metallic material. According to the invention, the internal reinforcement is inserted inside the amalgam still in its pasty state before moulding.

Though it is clear that the granules composing the traffic- and parking-preventing element 1 produced according to the process of the present invention could be derived from any type of rubber suitable for such purpose, preferably they are deriving from recycled tires (SBR) that are cleaned from ply, iron and other residuals and triturated. Obviously, the size of the rubber granules can be the most various, resulting in different levels of porosity and/or surface roughness of the traffic- and parking-preventing element 1. In particular, the Applicants have found that the mean size of the rubber granule should be preferably included between 0.5 mm and 13 mm, still more preferably included between 0.8 mm and 10 mm.

Obviously, the weight-increasing inert material could be of any type and/or nature that allows its mixing, amalgam and moulding with the other components of the traffic- and parking-preventing element 1. In general, the weight-increasing inert material will have a specific weight greater than the weight of the rubber granules. In particular, the weight-increasing inert material could be of a granular shape, such as sand, of an heterogeneous form, such as for example metal filings. Anyway, preferably, the weight-increasing inert material is composed of cobblestones of various nature, that are one of the most inexpensive and efficient solutions for realising the traffic- and parking-preventing element 1 produced according to process of the present invention.

Obviously, the polyurethane resin can be of any type and/or nature suitable for the purpose of the present invention. In particular, anyway, the polyurethane resin is preferably an isocianate.

The traffic- and parking-preventing element 1 could furthermore be equipped, on an upper portion thereof, with a hole 3, possibly threaded inside, to allow gripping of at least one eyelet with a similarly threaded hook, adapted to allow lifting, handling and laying the traffic- and parking-preventing element 1. Preferably, the hole 3 has a diameter D_{F} included between 7 cm and 9 cm.

The final shape of the traffic- and parking-preventing element 1 can obviously be various. Merely as an example, FIG. 1 shows a traffic- and parking-preventing element 1 having standard shapes and sizes required by Italian Laws, and it appears as a cylindrical body tapered as a dome in its upper part, in the centre of which the hole 3 is obtained.

The realisation of a traffic-and parking-preventing element 1 according to the process of the present invention having an approximate weight included between 100 kg and 115 kg, a height H included between 46 cm and 48 cm, a diameter D_{B} of the base 2 included between 46 cm and 48 cm, requires the use of an amount Q₁ of rubber granules preferably included between 40 kg and 60 kg and an amount Q₂ of weight-increasing inert material preferably included between 50 Kg and 70 Kg.

## Claims

1. Process for producing a traffic- and parking-preventing element (1) composed of a solid body equipped with at least one bearing base (2), said solid body being formed of at least one amalgam moulded in a solid form and composed of a mixture of rubber granules, of at least one polyurethane resin and of at least one weight-increasing inert material, said amalgam comprising at least one internal reinforcement structure, the mean size of said rubber granule being included between 0.5 mm and 13 mm, more preferably included between 0.8 mm and 10 mm, the process comprising the steps of:
a) providing an amount Q₁ of said rubber granules, said amount Q₁ being included between 40 kg and 60 kg;
b) providing an amount Q₂ of said weight-increasing inert material, said amount Q₂ being included between 50 kg and 70 kg, said weight-increasing inert material having a specific weight greater than the weight of said rubber granules;
c) forming an amalgam by mutually mixing said rubber granules and said weight-increasing inert material adding said at least one polyurethane resin;
d) filling at least one die with said amalgam, said step of filling comprising the substep of inserting said at least one internal reinforcement structure inside said amalgam;
e) moulding said amalgam to obtain said traffic- and parking-preventing element (1), said step of moulding comprising the substep of heating said die at a temperature included between 110°C and 170°C; and
f) extracting said traffic- and parking-preventing element (1) from said die.

2. Process according to claim 1, **characterised in that** step c) comprises the substep of adding at least one colouring paste inside said amalgam.

3. Process according to claim 1, **characterised in that** said polyurethane resin is an isocianate.

4. Process according to claim 1, **characterised in that** said internal reinforced structure is metallic.

5. Process according to claim 1, **characterised in that** said internal reinforcement structure is a cage.

6. Process according to claim 1, **characterised in that** said internal reinforcement structure is of a trellis type.

7. Process according to claim 1, **characterised in that** said weight-increasing inert material is sand.

8. Process according to claim 1, **characterised in that** said weight-increasing inert material are metal filings.

9. Process according to claim 1, **characterised in that** said weight-increasing inert material are cobblestones.

10. Process according to claim 1, **characterised in that** the traffic- and parking-preventing element is equipped with at least one hole (3) arranged on an upper portion of the element (1).

11. Process according to claim 10, **characterised in that** said hole (3) is internally threaded.

## Patentansprüche

1. Herstellungsverfahren eines Verkehrs- und Parkpfostens (1), der aus einem Festkörper besteht, welcher mit mindestens einer Stützbasis (2) ausgestattet ist, der genannte Festkörper ist aus mindestens einem Amalgam gebildet, das in fester Form gedruckt ist und aus einer Mischung aus Gummigranulaten, aus mindestens einem Polyurethanharz und mindestens einem inerten Beschwerungsmaterial zusammengesetzt ist, das genannte Amalgam schließt mindestens eine interne Verstärkungsstruktur ein, die durchschnittliche Dimension des genannten Gummigranulats liegt zwischen 0,5 mm und 13 mm, vorzugsweise zwischen 0,8 mm und 10 mm, das Verfahren schließt folgende Phasen ein:
a) Eine Menge Q₁ der genannten Gummigranulate liefern, die genannte Menge Q₁ liegt zwischen 40 kg und 60 kg;
b) Eine Menge Q₂ des genannten inerten Beschwerungsmaterials liefern, die genannte Menge Q₂ liegt zwischen 50 kg und 70 kg, das genannte inerte Beschwerungsmaterial hat ein spezifisches Gewicht, das größer als das Gewicht der genannten Gummigranulate ist;
c) Ein Amalgam bilden, indem die genannten Gummigranulate und das genannte inerte Beschwerungsmaterial miteinander vermischt werden mit Hinzufügung des genannten mindestens einem Polyesterharzes;
d) Mindestens eine Form mit dem genannten Amalgam füllen, die genannte Füllphase schließt die Unterphase ein, die genannte mindestens eine interne Verstärkungsstruktur in das genannte Amalgam einzuführen;
e) Das genannte Amalgam drucken, um den genannten Verkehrs- und Parkpfosten (1) zu erhalten, die genannte Druckphase schließt die Unterphase der Erhitzung der genannten Form auf eine Temperatur zwischen 110 °C und 170 °C ein; und
f) den genannten Verkehrs- und Parkpfosten (1) aus der genannten Form herausnehmen.

2. Verfahren gemäß Patentanspruch 1, das **dadurch gekennzeichnet ist, dass** die genannte Phase c) die Unterphase der Hinzufügung von mindestens einer Farbpaste in das genannte Amalgam einschließt.

3. Verfahren gemäß Patentanspruch 1, das **dadurch gekennzeichnet ist, dass** das genannte Polyurethanharz ein Isocyanat ist.

4. Verfahren gemäß Patentanspruch 1, das **dadurch gekennzeichnet ist, dass** die genannte interne Verstärkungsstruktur aus Metall besteht.

5. Verfahren gemäß Patentanspruch 1, das **dadurch gekennzeichnet ist, dass** die genannte interne Verstärkungsstruktur ein Käfig ist.

6. Verfahren gemäß Patentanspruch 1, das **dadurch gekennzeichnet ist, dass** die genannte interne Verstärkungsstruktur eine Gitterstruktur ist.

7. Verfahren gemäß Patentanspruch 1, das **dadurch gekennzeichnet ist, dass** das genannte inerte Beschwerungsmaterial Sand ist.

8. Verfahren gemäß Patentanspruch 1, das **dadurch gekennzeichnet ist, dass** das genannte inerte Beschwerungsmaterial Metallspäne sind.

9. Verfahren gemäß Patentanspruch 1, das **dadurch gekennzeichnet ist, dass** das genannte inerte Beschwerungsmaterial Kieselsteine sind.

10. Verfahren gemäß Patentanspruch 1, das **dadurch gekennzeichnet ist, dass** der Verkehrs- und Parkpfosten (1) mit mindestens einer Bohrung (3) ausgestattet ist, die an seinem Oberteil angebracht ist.

11. Verfahren gemäß Patentanspruch 10, das **dadurch gekennzeichnet ist, dass** die genannte Bohrung (3) ein Innengewinde hat.

## Revendications

1. Procédure de production d'une borne de dissuasion (1) composée d'un corps solide doté au moins d'une base d'appui (2), ce corps solide est formé au moins d'un amalgame moulé sous forme solide et composé d'un mélange de granulés en caoutchouc, d'une résine polyuréthane au moins et d'un matériau inerte alourdissant au moins ; cet amalgame comprend au moins une structure de renfort interne ; la dimension moyenne des granulés en caoutchouc peut être comprise entre 0,5 mm et 13 mm, mais il est préférable qu'elle soit comprise entre 0,8 mm et 10 mm ; cette procédure comprend les phases suivantes :
a) fournir une quantité Q₁ de granulés en caoutchouc, cette quantité Q₁ est comprise entre 40 kg et 60 kg ;
b) fournir une quantité Q₂ de matériau inerte alourdissant, cette quantité à Q₂ est comprise entre 50 kg et 70 kg ; le matériau inerte alourdissant doit avoir un poids spécifique supérieur au poids des granulés en caoutchouc.
c) former un amalgame en mélangeant entre eux les granulés en caoutchouc et le matériau inerte alourdissant, en ajoutant au moins une résine polyuréthane ;
d) remplir au moins un moule avec cet amalgame ; la phase de remplissage comprend une sous-phase qui consiste à insérer la structure de renfort interne à l'intérieur de l'amalgame ;
e) mouler cet amalgame pour obtenir la borne de dissuasion (1) ; cette phase de moulage comprend une sous-phase qui consiste à réchauffer le moule à une température comprise entre 110°C et 170°C ; et
f) extraire du moule la borne de dissuasion (1).

2. Procédure, selon la revendication 1, **caractérisée en ce que** la phase c) comprend la sous-phase qui consiste à ajouter une pâte colorante dans l'amalgame.

3. Procédure, selon la revendication 1, **caractérisée en ce que** la résine polyuréthane est un isocyanate.

4. Procédure, selon la revendication 1, **caractérisée en ce que** la structure interne de renfort est métallique.

5. Procédure, selon la revendication 1, **caractérisée en ce que** la structure interne de renfort est une cage.

6. Procédure, selon la revendication 1, **caractérisée en ce que** la structure interne de renfort est du type à treillis.

7. Procédure, selon la revendication 1, **caractérisée en ce que** le matériau inerte alourdissant est composé de sable.

8. Procédure, selon la revendication 1, **caractérisée en ce que** le matériau inerte alourdissant est composé de limailles métalliques.

9. Procédure, selon la revendication 1, **caractérisée en ce que** le matériau inerte alourdissant est composé de galets de pierre.

10. Procédure, selon la revendication 1, **caractérisée en ce que** la borne de dissuasion (1) est dotée au moins d'un trou (3) situé sur une portion supérieure de la borne.

11. Procédure, selon la revendication 10, **caractérisée en ce que** le trou (3) est fileté à l'intérieur.
